

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## KRAFT-SIMULATING PULP AND PROCESS OF PRODUCING SAME

No Drawing.

Application filed July 1, 1925. Serial No. 40,958.

This invention has relation to a novel pulp product possessing physical characteristics and a chemical composition substantially similar to kraft or "sulphate" pulp but which, however, is produced according to the present invention by a process quite dissimilar to the kraft or "sulphate" process, so-called. For convenience of designation, I will hereinafter term the pulp produced in accordance with the present invention a "kraft-simulating pulp" in contradistinction to pulps produced by the kraft or "sulphate" process.

In order to give a better understanding of the present process and the kraft-simulating pulp product secured thereby, it is necessary to consider, in some detail, the subject matter of my application for United States Letters Patent, Serial No. 749,564, filed November 12, 1924. In that application I have disclosed a process for producing pulp characterized by its extraordinary high Mullen or bursting strength and light color. The salient feature of discovery outlined therein, generally stated, is that if wood chips (spruce, for example) are cooked in an acid sulphite solution in which the free  $\text{SO}_2$  and the combined  $\text{SO}_2$  are in substantially equal proportions by weight (or the free  $\text{SO}_2$  less in proportion than the combined  $\text{SO}_2$ ) but are present in sufficient quantity in solution to act upon the encrusting or cementitious content of the wood for a sufficient period of time in a closed digester at a temperature higher than that ordinarily employed in sulphite digestion, a pulp of extraordinary strength and light color is produced. In practising the process, I employ a sodium bisulphite solution (or an equivalent bisulphite solution of zinc, magnesium, potassium or other suitable metal) in which the combined  $\text{SO}_2$  and free  $\text{SO}_2$  are in substantially equal proportion, say 3% to 4% of each. The digestion of the chips is carried out in a closed digester at a temperature of 320° F. and a pressure of 75 to 95 pounds for about ten to eleven hours. After the completion of the digestion, the digester contents are blown into a suitable blow pit, the pulp is separated from the spent liquor and is

washed, and, if desired, "screened" as ordinarily.

The pulp which results in the practice of a "4-4" digesting process, that is, a process employing a digesting liquor having about 4% combined and 4% free  $\text{SO}_2$ , has longer fibers and a much greater strength than the ordinary or commercial form of sulphite pulp. It is comparable in average length of fiber and Mullen or bursting strength with kraft or "sulphate" pulp and is characterized by the presence of a fairly high lignin and a high pentosan content which doubtless impart thereto certain of the characteristics hereinbefore noted.

Due to such high ligneous and pentosan content, however, the pulp is difficult to bleach, requiring 30% to 50% of 35% bleach, based on the bone-dry weight of fiber, and such bleaching operation resulting in a product which has a materially lower pentosan and lignin content and accordingly a lower strength (one which is comparable to that of ordinary bleached sulphite pulp), so that ordinarily it would not be economical or expedient to produce a bleached product therefrom in competition with the usual sulphite pulp for the manufacture of high grade writing papers. Moreover, although the unbleached "4-4" pulp, as such, would be particularly applicable for producing heavy papers for use in the manufacture of bags, wrapping paper, etc., it is ordinarily unsalable for such because of its deficiency in tear test and because the trade generally associates heavy and strong papers with a kraft or brown color and are prejudiced as to the value and strength of a light-colored product for such usage.

I have discovered that if the light-colored pulp produced by a "4-4" acid sulphite digestion of raw cellulosic material is subjected to treatment at an elevated temperature in an alkaline solution of the proper strength for a sufficient period of time, the pulp undergoes a color change or "coloration", assuming a brownish color similar to kraft or "sulphate" pulp. In such treatment, the alkaline solution must be of sufficient strength to cause the coloration or color change sub-

stantially without affecting or changing the fiber strength of the pulp, or, in other words, without removing or reducing materially the pentosan content thereof, since otherwise its 5 most important "kraft-like" property of strength will have been destroyed. Moreover, in addition to causing a coloration of the pulp I have found that the alkali treatment tends to remove less-resistant beta and 10 gamma celluloses and also to impart a materially increased softness to the pulp which, when tested, accordingly, shows an increased tear test.

While I am unable to account precisely as 15 to the theory or mechanism of the chemical reaction causing the coloration, I have reason to believe that the alkaline agent probably reacts with the lignin and pentosan in the pulp to produce a kraft-brownish color or 20 reaction product. Such a conclusion appears logical in view of the analogous colored pulp products formed in alkaline digestion, as for example in the kraft or "sulphate" process and in the soda process. Whatever the ex- 25 planation or theory involved in such coloration be, by the practice of my invention I am enabled to produce a pulp which is sub-stantially similar to kraft in both chemical and physical behavior but by a combination 30 acid-alkali treatment radically dissimilar to the kraft process and having certain very im- portant advantages which will subsequently be pointed out.

In the manufacture of the pulp of the pres- 35 ent invention, the wood chips to be digested, spruce for example, are placed in a digester in an acid sulphite liquor having a relatively high combined  $\text{SO}_2$  content, say 3% to 4%, and cooked under the requisite temperature, 40 pressure, and time conditions hereinbefore indicated and more fully set forth in the co-pending application for the production of a pulp product characterized especially by its unusually high strength and pentosan con- 45 tent. In certain cases, however, it may be de- sirable to commence the digestion of the chips in an acid liquor containing, say, about 7% free  $\text{SO}_2$  and 4% combined  $\text{SO}_2$ , and relieve the digester of the excess free  $\text{SO}_2$  during the 50 early stages of the cook. Such procedure, while substantially equivalent to that out-lined, gives better penetration of the  $\text{SO}_2$  into the chips and tends to promote a more rapid and efficient liberation of fiber. I de- 55 sire to make it clearly understood that where a kraft-simulating pulp is the ultimate prod- uct aimed at, not only low-resinous woods such as birch, beech, maple and hemlock, but also resinous woods frequently employed in 60 the manufacture of kraft pulp, such as jack- pine, long leaf pine, etc., may serve as the raw cellulosic material. Any resinous or 65 gummy material in a resinous wood which might survive the "4-4" acid sulphite diges- 70 tion and which might ordinarily interfere

with paper-making operations on the Four-drinier wire or felt of the paper-making ma-chine is removed by the subsequent alkaline digestion.

Due to the higher combined  $\text{SO}_2$  content 75 than is ordinarily present in the cooking of sulphite pulp, the hydrogen ion concentra-tion or activity of free  $\text{SO}_2$  is suppressed suf- ficiently to avoid the usual rather drastic hydrolysis which occurs in the cooking of sulphite pulp. This results in a pulp of 80 greater average fiber length and a higher pentosan and ligneous content than ordinarily in sulphite digestion; that is, the pulp con-tains more of the fiber and is produced with a higher yield than if digested in an acid sul-phite liquor, wherein hydrolysis of the cel-lulose fiber occurs to a greater extent, or even in an alkaline liquor.

The foregoing analysis of what takes place 85 is substantiated by actual data. For ex- ample, in ordinary commercial operation with the usual acid bisulphite digesting liquor the yield is from 43% to 47% of the weight of the dry wood. In ordinary sulphate or soda di- 90 gestion the yield is from 40% to 47% of the weight of the dry wood, whereas in the "4-4" acid sulphite treatment, on the other hand, the yield is from 50% to 55%, thus permitting a subsequent alkaline digestion with the final 95 "kraft-simulating pulp" yield, being equal to about 85% of the "4-4" pulp yield, and the over-all yield from the wood chips being about equal to that obtained by the usual kraft process.

After the completion of the "4-4" acid di- 100 gestion, the pulp is separated from the spent liquor; is washed as by passage through a counter-current washer of the type described in U. S. Letters Patent No. 1,421,664 to Brown et al., dated July 4, 1922; and is preferably 105 screened, as ordinarily, by passage through the usual screens employed for pulp to remove shives, specks and other like foreign material. The washed pulp is then thickened, as on a wet machine, and is intimately admixed with a 110 alkaline solution, preferably caustic soda ( $\text{NaOH}$ ) or sodium sulphide ( $\text{Na}_2\text{S}$ ), to the consistency desired for carrying out the alka-line treatment. The pulp is digested in the 115 solution at an elevated temperature and is agi-tated or stirred during digestion so as to pro-mote a uniform reaction for a sufficient period of time to allow the brown coloration and a softening of the light-colored pulp to be com- 120 pleted. I have found it more economical and expedient to carry out the alkaline digestion in open tanks under atmospheric pressure and to maintain an elevated temperature by blow-ing live steam into the tanks, but I desire to 125 have it understood that the alkaline diges-tion may be carried out in closed digesters at high pressure and temperature and yield equally satisfactory results. The alkaline di- 130 gestion does not materially affect the strength

or pentosan content of the pulp; but merely causes a coloration thereof and imparts an increased tear test thereto. In the alkaline digestion of a "4-4" pulp produced from resinous woods, the resinous and gummy material which may have survived the "4-4" digestion is to a great extent removed so that trouble in subsequent paper-making operations is not encountered. After the brown coloration of the pulp has taken place to completion, the pulp is washed, as by passage through a counter-current washing machine of the type hereinbefore indicated. The spent liquor presents a yellowish or brownish 15 appearance and perchance a darker appearance in the case of highly resinous woods. The washed pulp presents an appearance not unlike that of ordinary or commercial kraft pulp.

20 The following example will suffice to give a more comprehensive description of a preferred method of procedure falling within the purview of the present invention so as to allow those skilled in the art to practice the same. In carrying out the alkaline digestion, the washed and preferably screened "4-4" stock from the acid sulphite digestion of wood chips is digested at a stock density of about 10% in a caustic soda solution containing at least about 3% to 4% and not more than about 10% to 12% caustic soda based on the dry weight of pulp. The pulp is digested in open tanks under atmospheric pressure at a temperature of about 180° to 212° F., preferably while being agitated, from two to seven hours, or until the desired reaction is produced in the pulp, the time required therefor depending upon the characteristics of the particular stock undergoing treatment and the temperature employed in digestion. A coloration and increase in tear test is produced by such alkaline digestion substantially without affecting the strength of the pulp. The digested pulp is finally washed free from alkali and may be employed in the production of high-grade heavy papers suitable for the manufacture of bags, wrapping paper and like products which not only approximate the physical and chemical composition of kraft 45 products but have the color thereof.

50 It is again to be emphasized that in the combination treatment of the present invention, the yield of kraft-simulating pulp obtained is at least equal to the yield of kraft pulp resulting from the digestion of wood chips in a kraft or "sulphate" liquor. A great advantage in the manufacture of my "kraft-simulating" pulp is that it can be made in any locality because of the use of 55 unobjectionable methods of manufacture. As is known, kraft pulp can only be made in sparsely settled communities removed from large cities due to the undesirable mercaptan odor arising from the recovery of chemicals or in the digesting process. My inven-

tion may be practiced in localities where ordinances exclude the kraft process, because of its freeness from objectionable mal-odors. Moreover, the kraft-simulating pulp may be produced economically because of the efficient chemical recovery cycles practiced in conjunction therewith and the high yield obtained. I present a comparative table, the figures therein being average or representative, which indicate the similarity between 75 my product and the usual kraft or "sulphate" pulp and also show the effect of the alkaline digestion on the characteristics of the "4-4" pulp.

|                                    | "4-4" pulp  | Kraft-simulating pulp or "4-4" pulp after alkaline treatment | Usual kraft or "sulphate" pulp | 80 |
|------------------------------------|-------------|--------------------------------------------------------------|--------------------------------|----|
| Strength (beaten)                  | 160-165     | 154-160                                                      | 155-160                        | 85 |
| Slowness (beaten)                  | 4.59-6 min. | 11.2-13 min.                                                 | 7-10 min.                      |    |
| Alpha cellulose                    | 84.38-85    | 89.41-90                                                     | 89.90                          |    |
| Fiber length (cm.)                 | .96         | .79-.85                                                      | .7-.90                         |    |
| Tear                               | 144-150     | 257-290                                                      | 220-245                        |    |
| Pentosan content                   | 6.0-7       | 5.61-6.5                                                     | 7-10                           |    |
| Pulp yield (based on initial wood) | 54-55%      | 45-46%                                                       | 42-45%                         | 90 |
| Color                              | Light       | Kraft-like                                                   | Kraft                          |    |

From the foregoing table, which represents the average of a number of tests, it will be seen that the kraft-simulating pulp yield is at least equal to that resulting from the kraft or "sulphate" process of digestion and that the strength, slowness, alpha cellulose content, fiber length, and color thereof are about equal to that of kraft. It is to be noted that the alkaline treatment only slightly lowers the pentosan content of the "4-4" pulp, which is a trifle lower than that of kraft pulp, and raises the alpha cellulose content thereof to that of kraft pulp, probably because of the removal of ligneous matter, less resistant celluloses and resinous material therefrom.

95 Before concluding, it may be stated that the results realized in the practice of the present invention cannot be obtained by an alkaline digestion of wood chips followed by a "4-4" treatment. The essential feature lies in the alkaline treatment subsequent to the "4-4" digestion.

#### What I claim is:

1. A process of producing a kraft-simulating pulp, which comprises digesting wood chips at elevated temperature and pressure in an acid sulphite liquor in which the free SO<sub>2</sub> and combined SO<sub>2</sub> are in approximately 100 equal proportions of 3% to 4% each, separating the resulting pulp from its digesting liquor, and digesting such predigested pulp in an alkaline cooking liquor.

115 2. A process of producing a kraft-simulating pulp, which comprises digesting wood chips at elevated temperature and pressure in an acid sulphite liquor in which the free SO<sub>2</sub> and combined SO<sub>2</sub> are in approximately 120 equal proportions of 3% to 4% each, separat-

ing the resulting pulp from its digesting liquor, and cooking such predigested pulp in a caustic soda solution containing from about 3% to 12% caustic soda, based on the dry weight of pulp.

In testimony whereof I have affixed my signature.

GEORGE A. RICHTER.